

Aug. 31, 1943.

A. S. HUNTER

2,328,074

MANUFACTURE OF TEXTILE YARN

Filed July 16, 1940

Fig. 1.



Fig. 2.



Inventor  
Archibald S. Hunter

By

*C. Ralph Snyder*

Attorney

## UNITED STATES PATENT OFFICE

2,328,074

## MANUFACTURE OF TEXTILE YARN

Archibald Stuart Hunter, Kenmore, N. Y., assignor to E. I. du Pont de Nemours & Company, Wilmington, Del., a corporation of Delaware

Application July 16, 1940, Serial No. 345,778

2 Claims. (Cl. 18—54)

This invention relates to the manufacture of textile yarn. More specifically, it relates to a process of producing novelty yarn composed of two or more strands of filaments, said strands having shrunk unequally during the production thereof to form a pebbly yarn structure.

Novelty yarns which are a composite of two or more single yarns of different lengths are known to the art. Such multiple yarns are produced by combining two or more single yarns having different shrinkage characteristics and thereafter subjecting the yarn to a shrinking treatment. In U. S. Patent No. 1,976,201, a method is described for producing multiple yarn from cellulose acetate, wherein two yarns coming from a spinning machine are subjected to different degrees of stretching, then are combined into one strand and finally thrown on a down-twister and collected on a bobbin. The degree of tension on one of the yarns is such that the yarn is stretched beyond its elastic limits. The composite yarn on the bobbin is subjected to the customary after-treatment procedure and then to a shrinking treatment. The filaments of the yarn which was subjected to the higher tension, will shrink to a greater degree and will, therefore, be shorter than those of the yarn which was subjected to the lower tension.

Novelty or composite yarns made from cellulose acetate according to the method described in U. S. Patent No. 1,976,201 do not possess a very great difference in length of the single yarn members. Yarn produced in accordance with this process, therefore, does not exhibit a definite pebbly or rippled effect. It is important to note that in yarns of this character, the component yarn which has been subjected to a tension beyond the elastic limit thereof exhibits the higher degree of shrinkage and becomes the core, or the shorter member, of the composite yarn.

It is an object of this invention to provide a process for producing a rippled novelty yarn wherein the ripples are quite pronounced.

Another object of this invention is to provide a process for the production of a rippled, or pebbly, novelty yarn during the conventional steps of spinning and purification, without the necessity of having additional shrinking and drying procedures.

It is a further object of this invention to provide a yarn which when woven into fabric will give depth to the fabric, thereby eliminating the uninteresting flat appearance common to most fabrics.

Other objects of this invention will appear hereinafter.

The objects of this invention are accomplished, in general, by spinning several regenerated cellulose yarns, or similar acid coagulated yarns, under different tensions but without exceeding the elastic limit of the yarn, combining the yarns while still in the gel state and twisting the several yarns, for example, into a bucket in accordance with the bucket spinning process. The composite yarn is then dried while maintaining the same free from tension.

By a "gel" yarn is meant a freshly spun coagulated yarn which has never been dried and which contains a large amount of water. Gel shrinkage of a yarn may be described as the amount a gel yarn will shorten when allowed to dry while under no tension. When a yarn is dried while under tension either in the form of a bucket cake or on a bobbin, it can shrink only to a small degree. Since after drying in this manner, the yarn is still in a strained condition, it still retains the capacity to shrink. It possesses, therefore, residual shrinkage which may be measured or determined by subjecting the yarn to a boil-off procedure which comprises, for example, treatment of the yarn with a hot bath and permitting the same to dry without restraint.

For convenience, the present invention will be described with particular reference to the production of regenerated cellulose yarn from viscose. The present invention is not limited thereto, but is applicable generally to the production of yarn from aqueous cellulosic filament-forming solutions which may be coagulated in the acid coagulating bath, for example, lowly etherified cellulose compositions such as ethyl cellulose. The invention is also applicable to the production of yarn by the cuprammonium process.

Referring to the accompanying drawing wherein Fig. 1 is a diagrammatic illustration of one arrangement for carrying out the tension spinning and doubling steps of this invention, and Fig. 2 is a diagrammatic illustration of an arrangement for carrying out the tension-free drying step, this invention may, for example, be carried out as follows: Two yarns A and B freshly spun from spinnerets 1 and 2 respectively, into a spinning or coagulating bath 3 are, while still in the gel state, subjected to different tensions by passing one yarn over the enlarged portion, and the other yarn over the reduced portion of a conventional roll 4, and then passing both yarns over a drawing roll 4' which is of the same diameter as that of the enlarged portion of roll

4 and which is driven at the same speed where-  
by yarn B is subjected to the requisite stretch.  
Thereafter the yarns are combined in guide 5  
and fed into bucket 6, preferably at equal rates  
of speed, during which procedure the two yarns  
are twisted together and collected as a cake 7.  
While the combined yarn is still in the gel state,  
it is wound on reel 8 from cake 7 to form skeins.  
The skeins are allowed to dry freely while under  
no tension. The ripple develops as one compo-  
nent shrinks on drying more than the other.  
Any other suitable expedient for spinning one  
yarn at a higher tension than the other may of  
course be employed.

Surprisingly, the yarn which was spun at the  
lower tension shrank to a considerably greater  
degree than the other yarn. This component  
was, therefore, shorter in the shrunken yarn and  
consequently constitutes the core, while the other  
yarn spun under the higher tension forms the  
ripples and gives the novelty effect.

The following examples illustrate several de-  
tailed processes for carrying out the present in-  
vention.

#### Example I

Viscose was spun through two identical spin-  
nerets mounted side by side in a coagulating and  
regenerating bath to form yarns which were con-  
tinuously removed, combined into one strand,  
and collected on a bobbin at a take-up speed of  
2,000 inches per minute. The spinnerets con-  
tained 40 holes each. The diameter of the holes  
was 0.0035 inch. The yarn from one of the spin-  
nerets, yarn A, was a 370-denier, 40-filament yarn  
and was spun with a 6-inch bath travel. The  
other yarn, yarn B, was a 370-denier, 40-filament  
yarn and was spun with a 90-inch bath travel.  
The combined yarn collected on the bobbin was  
washed acid-free on the bobbin and while still  
in the wet gel state, thrown on a downtwister  
which applied 3 turns per inch to the yarn. The  
gel yarn was immediately reeled to skeins and  
while in a completely relaxed state, was allowed  
to dry. During the drying, yarn component A  
which was spun under low tension decreased in  
length 9.8%, while yarn component B which  
was spun under a higher tension decreased in  
length 4%. The differential shrinkage obtained  
was therefore 5.8%. Because of the shrinkage  
difference, yarn component A became shorter  
than the other, said component becoming the  
base yarn, while yarn component B was loosely  
twisted thereabout.

#### Example II

Two yarns were spun as follows: Yarn A which  
was a 200-denier, 40-filament yarn was produced  
by spinning viscose into a coagulating bath using  
a 6-inch bath travel and winding the same on a  
bobbin by the conventional "bobbin-spinning"  
process. Yarn B which was a 300-denier, 120-  
filament yarn and which contained 4 8 turns  
per inch was produced by spinning viscose into  
a coagulating regenerating bath using 100 inches  
bath travel and collecting in a bucket by the  
"bucket-spinning" process. The two yarns were  
subjected to the usual after-treatments such as  
washing, desulfuring and bleaching, in that form.  
The two yarns were combined by twisting to-  
gether on a downtwister while still in the wet gel  
state. The combined yarn was then reeled to  
skeins and dried in the relaxed state. Yarn A  
which was spun under low tension possessed a  
gel shrinkage on drying of 6.2%, while yarn B  
had a shrinkage of 2%, giving a differential

shrinkage of 4.2%. A yarn effect similar to that  
of Example I was obtained.

#### Example III

5 Yarn B of Example II while in the gel state  
was combined on a downtwister with yarn made  
as follows: A high salt index viscose, said index  
being 8, modified with 5% sodium sulfate was  
spun into a coagulating regenerating bath to give  
10 a yarn of 370-denier, 40-filament, using a 6-inch  
bath travel and collected on a bobbin. The  
combined yarns after purification were reeled to  
skeins and allowed to dry. The gel shrinkage of  
the yarn spun from the high index viscose was  
15 12.1%, while that of yarn B was 2%, giving a  
differential shrinkage of 10.1%. A yarn having  
a pronounced ripple effect was obtained, the  
effect being produced by the long and short com-  
ponents thereof.

#### Example IV

20 Two yarns having different filament sizes and  
spun under different tensions were produced as  
follows. Yarn A which was a 370-denier, 10-fila-  
ment yarn was spun through a spinneret having  
25 10 holes, each hole being 0.012 inch in diameter,  
using a 6-inch bath travel and collected on a  
bobbin. Yarn B which was a 70-denier, 40-fila-  
ment yarn was spun through a spinneret having  
30 40 holes, each hole being 0.0035 inch in diameter,  
using a 50-inch bath travel and collected on a  
bobbin. The two yarns were washed and purified  
35 on the bobbin and thrown on a downtwister  
which applied 3 turns per inch to the yarn. The  
wet yarn was immediately reeled to skeins and  
allowed to dry in a relaxed form. Yarn A which  
40 contains the large filaments possessed a shrink-  
age on drying of 6.9%, while yarn B containing  
filaments of small size spun under a higher ten-  
sion possessed a shrinkage on drying of 2.4%,  
giving a differential shrinkage of 4.5%. A yarn  
45 of the nature described in the previous examples  
was obtained.

Preferably the component yarn which is spun  
with a high tension is spun with a tension two  
50 or more times the spinning tension of the  
other component yarn or yarns. The high dif-  
ferential shrinkage of the component yarns is  
believed due to the fact that they are com-  
bined to form a composite yarn while still in  
55 the wet gel state. The yarn according to this in-  
vention is distinguished from that of the prior  
art in that the base yarn or the short yarn is the  
one which was spun under the lower tension.  
The present invention is further distinguished by  
60 the fact that the gel shrinkage between yarns  
spun under different tensions differs to a greater  
degree than the residual shrinkage of the same  
yarn. By this fact, it has been possible to obtain  
65 novelty yarns having a more pronounced ripple  
effect than was produced by the prior art. For  
the production of a satisfactory novelty yarn in  
accordance with the present invention, it is es-  
sential that the shrinkage difference between the  
70 yarns must be in excess of 3%. For the best re-  
sults, the shrinkage differential between the two  
yarns should be from 5% to 10%, or even higher.

The gel shrinkage of a yarn increases with an  
increase in filament denier, an increase in the  
total denier, and with a decrease of spinning ten-  
sion. If two gel yarns are combined which have  
75 a wide difference in filament denier, a wide dif-  
ference in total denier, and which were spun un-  
der widely different tensions, a high gel shrink-  
age differential will be obtained. Two yarns,  
which are identical with the exception that one

has been spun under a much higher tension than the other, will give a satisfactory shrinkage differential though not as high as when all controlling factors have been utilized.

In the above examples, several ways of producing the novelty yarn of this invention have been described. The invention is not to be limited to these examples since it is possible to vary the conditions of spinning the yarn and still obtain yarns having different gel shrinkage values. For example, a different denier yarn may be obtained by maintaining all conditions the same, with the exception of the pump delivery which may be increased for one of the yarns. The denier may be further increased by slowing down the take-up of the yarn. The denier differential may be further effected by using spinnerets having large orifices.

In the examples, processes have been described in which the yarns when reeled to skeins were acid-free and in some cases purified. It is to be understood that satisfactory results, and in some cases more satisfactory results may be obtained by a process in which acid gel yarns are reeled to skeins and dried in the relaxed state.

The spinning tension to which the yarn is subjected may be controlled by the length of bath travel. It may be further effected by the use of a series of rollers in the bath around which the yarn must travel. Additional tension may be applied by providing said rollers with vanes.

This invention has been described in terms of a yarn containing two components, but it is obvious that three, or in some cases four or more component yarns may be twisted together to produce the composite yarn.

The present invention is described with particular reference to the production of regenerated cellulose from viscose solutions. The invention is, however, generally applicable to the production of yarn from any aqueous cellulosic solution which is coagulable in an acid coagulating bath. Production of cellulosic yarns from aqueous solutions with the coagulation of the aqueous solutions in an acid or neutral bath will be referred to herein as a "wet spinning" process.

In the process described in the examples, the yarn was reeled to skeins and allowed to dry while relaxed. The process is not to be limited, however, to drying the yarn in skein form as satisfactory results will be obtained by any process in which the yarn is dried while relaxed.

The process of this invention makes it possible to produce a novelty rippled yarn during the standard steps of spinning and purification. It is not necessary, therefore, to provide more than one drying, stretching or shrinking procedure, as would be the case if the novelty effect were to be produced by the residual shrinkage of the yarn.

The yarns may be knitted or woven in the customary manner to give fabrics having unusual properties. The kinky, rippled or pebbly nature of the yarn gives an increased loft to fabric made therefrom. The component members of the yarn which are spun at different tension, possess different dyeing characteristics and, therefore, may provide a novelty dyeing effect in the fabric. The fabrics are full, voluminous, and possess a less slippery hand. The kinky, rippled yarn of this invention possesses the further advantage over the prior art yarns in that the ripples are permanent and will not be pulled out on stretching.

Since it is obvious that many changes and modifications can be made in the detailed processes above described without departing from the nature and spirit of the invention, it is to be understood that the invention is not to be limited except as set forth in the appended claims.

I claim:

1. In the method of making a rippled composite yarn by wet spinning, at different spinning tensions, a plurality of yarns of different deniers composed of artificial cellulosic filaments, the improvements comprising applying to the yarn of least denier a spinning tension at least two times the spinning tension of the yarn of largest denier, doubling said yarns, and drying the doubled yarns while they are still in the gel state by supporting them in a loose condition free from tension.

2. In a method of making a rippled composite yarn by wet spinning, at different spinning tensions, a plurality of yarns of different filament deniers composed of artificial cellulosic filaments, the improvements comprising applying to the yarn of least filament denier, a spinning tension at least two times the spinning tension of the yarn of largest filament denier, doubling said yarns, and drying the doubled yarns while they are still in the gel state by supporting them in a loose condition free from tension.

ARCHIBALD STUART HUNTER.